

1

3,234,054  
PROCESS FOR PREPARING ALUMINUM  
BASE ALLOY

Philip R. Sperry, North Haven, Conn., assignor to Olin Mathieson Chemical Corporation, a corporation of Virginia  
No Drawing. Filed Aug. 5, 1964, Ser. No. 387,791  
9 Claims. (Cl. 148—11.5)

The present application is a continuation-in-part of United States patent application Serial No. 227,000 by P. R. Sperry, filed September 28, 1962, now abandoned.

The present invention relates to a process for obtaining an aluminum base alloy containing silicon and magnesium and the alloy obtained thereby. More particularly, the present invention relates to a process for obtaining an extruded aluminum base alloy as above wherein the alloy obtained thereby is characterized by improved strength characteristics while retaining the excellent characteristics desired in alloys of this type.

Various aluminum base alloys containing magnesium and silicon are well known, such as, for example, aluminum alloy 6063 containing from 0.20 to 0.60 percent silicon, from 0.45 to 0.90 percent magnesium and the balance essentially aluminum and aluminum alloy 6061 containing from 0.40 to 0.80 percent silicon, from 0.80 to 1.2 percent magnesium, from 0.15 to 0.40 percent copper, from 0.15 to 0.35 percent chromium and the balance essentially aluminum. These alloys find wide application, for example, in the preparation of extruded products. That is, products wherein the alloy is shaped by forcing the heat softened alloy through dies by pressure. These alloys are in general characterized by a range of moderate strength properties accompanied by fair to good corrosion resistance, anodizability, formability, and weldability. In order to develop the strength properties of these alloys to the maximum degree, it is generally necessary to perform costly separate heat treatments after extrusion. For example, in order to develop the full strength properties of alloy 6061, which is the stronger of the two alloys, there is required a solution heat treatment of 970° F. for about one hour, followed by water quenching and then artificial aging at 320° F. for 18 hours (T6 temper). Alloy 6061 does not have good appearance after anodizing and does not resist corrosion as well as 6063.

The maximum strength properties of alloy 6063 are developed by forced air cooling after extrusion ("press quenching"), followed by artificial aging at 350° F. for 8 hours (T6 temper). Alternatively, for a somewhat reduced strength at lower cost, 6063 is artificially aged at 365° F. for 5 hours (T5 temper). The maximum strength of 6063 is considerably less than alloy 6061.

What is desired in alloys of this type is an alloy and a method of manufacture which would:

- (1) Develop at least the minimum required properties for 6063-T5 by natural aging, but without any artificial aging heat treatment; and
- (2) develop the high strength properties of 6061-T6 simply by press quenching and artificial aging, without the need of a separate solution heat treatment.

Both of these goals should be accomplished while retaining the excellent extrudability, good anodizability and good corrosion resistance of 6063.

Accordingly, it is a principal object of the present invention to provide a process for treating aluminum base alloys containing silicon and magnesium and to provide an improved alloy obtained hereby, especially an alloy which attains the foregoing desirable goals.

It is a further object of the present invention to provide a process and alloy as aforesaid which obtains improved strength characteristics while retaining the highly

2

desirable characteristics of this type of alloy, namely in particular good corrosion resistance, anodizability, appearance, formability, uniformly fine grain structure, and weldability.

It is a still further object of the present invention to provide a simple and expeditious process which accomplishes the aforesaid objects conveniently and at a commercially competitive cost.

Further objects and advantages of the present invention are apparent hereinafter.

In accordance with the present invention, it has now been found that the foregoing objects and advantages as well as others may be readily accomplished. Briefly, the process of the present invention comprises:

(a) Providing an aluminum base alloy containing from 0.60 to 0.90 percent silicon, from 0.40 to 0.60 percent magnesium and the balance aluminum, wherein said silicon and magnesium are uniformly distributed throughout the said alloy, preferably by an elevated temperature homogenization treatment;

(b) Heating said alloy to a temperature of at least 970° F.;

(c) Holding said alloy at said temperature of at least 970° F. for at least 2 minutes;

(d) Extruding said alloy at a temperature in excess of 950° F., i.e., before the surface temperature of the billet has dropped below 950° F.; and

(e) Rapidly cooling said extruded alloy to a temperature of at least 350° F. in at most 4 minutes.

It has been found that the alloy treated in accordance with the foregoing process develops critically improved properties. Upon natural aging after extrusion it develops properties exceeding the minimum guaranteed for 6063-T5. In addition, however, it has been further found that still greater improvement is obtained when the alloy is thermally artificially aged subsequent to the rapid cooling step.

Thus, the improved alloy of the present invention is a high strength extruded aluminum base alloy containing from 0.60 to 0.90 percent silicon, from 0.40 to 0.60 percent magnesium, and the balance aluminum, wherein the silicon and magnesium are retained in solid solution, said alloy being in the extruded condition. Generally, the minimum strength properties of the extrusion of the present invention are: tensile strength 26,000 p.s.i.; and yield strength 16,000 p.s.i.

The alloy to which the present invention relates is an aluminum base alloy containing from 0.60 to 0.90 percent silicon, from 0.40 to 0.60 percent magnesium and the balance aluminum. Preferably when the alloy is in the T-42 temper (naturally aged) it contains from 0.75 to 0.85 percent silicon and from 0.50 to 0.60 percent magnesium. Preferably when the alloy is in the T-5 temper (artificially aged) it contains from 0.70 to 0.85 percent silicon and 0.45 to 0.60 percent magnesium. Preferably the total magnesium plus silicon content should range from 1.3 to 1.5 percent and the preferred ratio of silicon to magnesium in the aluminum alloy is from 1.30:1 to 1.5:1, with an optimum total magnesium plus silicon content being about 1.4 percent in conjunction with an optimum silicon to magnesium ratio of 1.4:1. It has been found that the foregoing composition is preferred and provides the optimum characteristics of strength, anodizability, corrosion resistance, formability and extrudability.

Naturally, the present invention contemplates conventional impurities common for alloys of this type. This is important since it indicates that the improved properties of the alloys in the present invention are obtainable with normal commercial impurity materials. For example, normal impurities comprise: 0.35 percent maximum iron; 0.10 percent maximum copper; 0.10 percent maximum manganese; 0.10 percent maximum chromium; 0.10 per-

cent maximum zinc; 0.10 percent maximum titanium; and 0.05 percent maximum each of other elements, the total of which is a maximum 0.15 percent.

The manner of melting and casting the alloy is not especially critical and conventional methods of melting and casting may be conveniently employed. Before the process of the present invention is performed, however, it is important to uniformly distribute the silicon and magnesium throughout the matrix of the alloy. This may be done in any desired manner, for example, it may be done preferably by a homogenization heat treatment subsequent to the casting operation. In fact, the preferred method for uniformly distributing the silicon and magnesium throughout the alloy is by homogenizing the alloy at a temperature of from 970 to 1100° F. for from 4 to 20 hours. In the preferred embodiment, the homogenization treatment is followed by cooling to room temperature in any desired manner.

The cooling of the cast ingots subsequent to the homogenization treatment is normally rather slow because of the large mass of material involved. Consequently much of the soluble alloying constituent necessarily is precipitated out of solution during the slow cooling which must follow the homogenization treatment. In accordance with the present invention, this precipitated material must be completely redissolved prior to extrusion in order to develop full strength and hardness in the present alloy. Naturally, where the silicon and magnesium are dissolved as well as uniformly distributed throughout the matrix of the alloy, it is unnecessary to redissolve these materials. However, it is judicious to perform the redissolving step in order to insure the dissolution of all of these materials.

In accordance with the present invention, therefore the alloy should be heated to a temperature of at least 970° F. and held at that temperature for at least 2 minutes. The temperature 970° F. is the solution temperature for the soluble magnesium and silicon components and the time at that temperature must be sufficient to dissolve all the soluble magnesium and silicon components. The time period of at least 2 minutes is normally the minimum requirement. The upper temperature is governed by avoiding partial melting and excessive oxidation; however, generally a temperature of 1100° F. is not exceeded. The minimum time of treatment is not especially critical. It is noted in this regard that optimum properties are developed only if all of the alloy is retained at at least 970° F. and at least 2 minutes, in other words, optimum results will be obtained only if the temperature at the center of the billet reaches 970° F. or higher and is kept from falling below 970° F. for 2 minutes prior to extrusion.

Subsequent to the heating and holding step the extrusion billet of the desired alloy is inserted into the extrusion press before the surface temperature has dropped below 950° F. and the extrusion is then made immediately. Naturally, in view of the foregoing, the alloy should not be cooled below 950° F. prior to extrusion but should be extruded directly after the heating and holding steps. The upper temperature is dependent upon surface appearance and temperature effects on the extrusion tools; generally, however, a temperature of less than 1050° F. is used.

Subsequent to extrusion, it is critical that the extruded alloy be rapidly cooled in order to eventually obtain the maximum strength properties. The effect of the rapid cooling is to retain the soluble magnesium and silicon constituents in solid solution. It has been found that the critical cooling step is to bring the extruded alloy down to a temperature of 350° F. or lower in 4 minutes or less. Naturally it is preferred that the alloy be cooled more rapidly than the foregoing minimum cooling rate. More rapid cooling gives better ductility combined with high strength.

This rapid cooling rate may be accomplished in extrusion sections up to about 1/4 of an inch in thickness by

air cooling using appropriately placed fans in order to provide some continuous replacement of air. In sections in excess of 1/4 of an inch in thickness, it is generally desirable to obtain a suitable cooling rate by passing the extrusion through a water spray quench, if this can be done without excessive distortion of the extruded shape.

The resultant as extruded alloy thus is a moderate strength extruded aluminum base alloy and has been found to have excellent physical properties, such as formability, weldability, corrosion resistance, and anodizability. It is further noted that the resultant alloys obtain improved strength levels without degradation of the aforementioned desirable characteristics of alloys of this type.

A still further and in fact surprising finding of the present invention is the level of additional improvement obtained subsequent to the rapid cooling step by thermally artificially aging the extrusion. The preferred manner of this artificial aging is to maintain the extrusion for from 15 minutes to 9 hours at a temperature of from 200 to 410° F. and preferably at about 350° F. and from 4 to 8 hours. With the foregoing artificial aging treatment the alloy of the present invention attains strength properties equivalent to those of the more expensive alloy 6061 and in fact exceeds by far the strength properties of alloy 6063 in the T5 or artificially aged condition. These advantages are obtained with no sacrifice in the other desirable characteristics of this type of alloy, such as, for example, extrudability, anodizability, finishing characteristics, corrosion resistance or weldability. In addition, the advantages of the present invention have been obtained without a separate solution heat treatment step as is required for 6061-T6. It is also possible to artificially age the alloy of the present invention to the typical strength level of alloy 6063 in the T5 or artificially aged condition and to obtain a considerably higher tensile elongation, hence ductility. Thus the present alloy offers an extremely versatile range of properties heretofore unattained in an inexpensive alloy.

For example, when the alloy of the present invention is artificially aged at 310° F. for 2 hours, it will have yield and ultimate strengths somewhat higher than those for alloy 6063 in the T5 or artificially aged condition, while its elongation will be 18 percent instead of the 12 percent typical of alloy 6063 in the T5 or artificially aged condition. This characteristic would allow more forming to be done on the alloy of the present invention than on alloy 6063-T5 while maintaining a better than average strength level.

In addition the alloy of the present invention has other highly beneficial and distinguishing characteristics. The alloy of the present invention shows minimum distortion upon completion of extrusion and therefore the subsequent straightening required is quite small; whereas 6061 distorts appreciably and requires fairly extensive subsequent straightening. This advantage of the present alloy economizes the extrusion operation and also permits better dimensional control of complex shapes. In addition, the present alloy has good properties on porcelain enameling, superior to the conventionally used 6063. In addition, the electrical characteristics of the present alloy are good, i.e., the present alloy is a high strength, moderate conductivity alloy. For example, the present alloy has an electrical conductivity of 50 percent IACS at peak hardness equivalent to 6061-T6 which has a conductivity of 43 percent IACS. Alloy 6063 has considerably lower hardness.

The present invention will be more readily apparent from a consideration of the following illustrative examples.

#### EXAMPLE I

Ingots were prepared in a conventional manner summarized as follows. Melting and alloying was carried out in a gas-fired, open hearth furnace. After alloying the melt was degassed by gaseous chlorine fluxing for 20

minutes. The average pouring temperature was 1360° F. The average casting speed was 5" per minute and the metal head was maintained between 2.5 and 3".

The composition of the alloy prepared was as follows: 0.55 percent magnesium; 0.82 percent silicon; 0.16 percent iron; 0.02 percent zinc; and traces of copper, manganese and chromium.

#### EXAMPLE II

The silicon and magnesium in the cast ingots were uniformly distributed throughout the matrix by the following homogenization procedure. The ingots were heated so that the entire furnace load reached a temperature exceeding 970° F. within the first 8 hours. They were then held for an additional 6½ hours, during which time no portion of the furnace load exceeded 1095° F. Finally, the entire load was removed from the furnace and cooled in air which took about 6 hours.

#### EXAMPLE III

The ingots prepared in accordance with Examples I and II were subjected to three different types of treatments, identified below as Treatment A, Treatment B and Treatment C.

*Treatment A.*—The ingots were placed in a gas-fired, continuous feed furnace maintained at 1000° F. and retained therein for 20 minutes. Upon exiting from the furnace, the surface of the alloy was allowed to cool to 960° F. The ingots were then extruded, with the surface temperature being 930 to 990° F. upon exiting from the extrusion press, followed by rapidly cooling to room temperature, with a temperature of 350° F. being attained in 4 minutes or less.

*Treatment B.*—The ingots were placed in an electrical induction heater set to give a heating time of ½ minute at 990–1000° F. Upon exiting from the heater the surface temperatures of the billets was allowed to cool to three different levels as follows:

Treatment B-1, cooled to 920° F.;  
Treatment B-2, cooled to 950° F.; and  
Treatment B-3, cooled to 980° F.

The ingots were then extruded, with corresponding surface temperatures obtained upon exiting from the extrusion press as follows:

B-1, surface temp., 900–970° F.;  
B-2, surface temp., 940–1000° F.; and  
B-3, surface temp., 950–1020° F.

Following extrusion all alloys were rapidly cooled to room temperature, with 350° F. being attained in 4 minutes or less.

*Treatment C.*—Ingots were treated in a manner after Treatment B, except that the electrical induction heater was set to give a heating time of 2 minutes and upon exiting from the heater the surface temperature of the billet was allowed to cool to a temperature not below 950° F.

#### EXAMPLE IV

The properties of the extrusions obtained in Example III were determined as follows: the tensile strength was determined; the yield strength at 0.2 percent offset; and elongation in 2 inches. The results are given in the following table. These are compared with the minimum properties of the comparable alloy 6063-T5.

Table I

| Extrusion                  | Tensile Strength in p.s.i. | Yield Strength in p.s.i. | Elongation in Percent |
|----------------------------|----------------------------|--------------------------|-----------------------|
| Example III, Treatment A   | 30,300                     | 18,300                   | 18.3                  |
| Example III, Treatment B-1 | 29,900                     | 15,100                   | 21.7                  |
| Example III, Treatment B-2 | 30,600                     | 15,800                   | 22.3                  |
| Example III, Treatment B-3 | 30,800                     | 16,000                   | 22.1                  |
| Example III, Treatment C   | 33,000                     | 18,000                   | 21.5                  |
| Alloy 6063-T5              | 22,000                     | 16,000                   | 8                     |

The foregoing shows that in the treatment conditions of Example III, Treatment A, the heating time of 20 minutes was long enough to guarantee that all of the magnesium and silicon would be taken back into solution so that the minimum strength properties of alloy 6063-T5 are readily exceeded. However, the treatment conditions of Example III, Treatment B-1, B-2 and B-3, namely a heating time of ½ minute, was not long enough to guarantee that the minimum will be exceeded. But the treatment conditions of Example III, Treatment C was sufficient, namely 2 minutes.

In addition to exceeding the minimum strength characteristics of alloy 6063-T5, the alloys of the present invention have excellent elongation which enable them to be more readily formed than 6063-T5.

A further, and in fact quite surprising characteristic, was that the alloys of the present invention were found to have superior punching and blanking characteristics than 6063-T5. This is quite surprising in view of the higher ductility of the present alloy.

#### EXAMPLE V

The alloys treated in the manner of Examples I, II and III were artificially aged under varying conditions and tensile strength, yield strength and elongation determined. The results are compared with the minimum and typical properties of 6061-T6 and 6063-T5. The results substantiate that the alloy of the present invention is comparable in strength characteristics to the expensive 6061-T6 and far superior to 6063-T5. The results are given in the following table.

Table 2

| Alloy                     | Time and Temperature of Aging | Tensile Strength in p.s.i. | Yield Strength in p.s.i. | Elongation in Percent |
|---------------------------|-------------------------------|----------------------------|--------------------------|-----------------------|
| Example III, Treatment A. | 350° F. for 4 hours.          | 44,000                     | 39,500                   | 10                    |
| Example III, Treatment A. | 350° F. for 8 hours.          | 43,500                     | 40,000                   | 9                     |
| 6061-T6 Minimum           |                               | 38,000                     | 35,000                   | 10                    |
| 6061-T6 Typical           |                               | 45,000                     | 40,000                   | 12                    |
| 6063-T5 Minimum           |                               | 23,000                     | 16,000                   | 8                     |
| 6063-T5 Typical           |                               | 27,000                     | 21,000                   | 12                    |

In addition, the alloys of the present invention were formed to have extrudability comparable to or slightly better than 6063, and far better than 6061, which enabled complex shapes to be extruded with a minimum of distortion and good dimensional control.

#### EXAMPLE VI

The following additional properties of the alloys of the present invention were evaluated:

- (1) *Corrosion resistance.*—Either the natural or artificially aged alloy of the present invention were found to be superior to 6063 or 6061 as determined by immersion in a corrosive environment, e.g., sea water.
- (2) *Anodizability.*—Either the natural or artificially aged alloy of the present invention were found to have a pleasing and uniform appearance upon etching and anodizing by standard anodizing procedures; and
- (3) *Weldability.*—Either the natural or artificially aged alloy of the present invention were found to be readily weldable in a manner comparable to 6061 or 6063.

This invention may be embodied in other forms or carried out in other ways without departing from the spirit or essential characteristics thereof. The present embodiment is therefore to be considered as in all respects illustrative and not restrictive, the scope of the invention being indicated by the appended claims, and all changes which come within the meaning and range of equivalency are intended to be embraced therein.

What is claimed is:

1. The process which comprises:

- (a) providing an aluminum base alloy consisting essentially of from 0.60 to 0.90 percent silicon, from 0.40 to 0.60 percent magnesium and the balance aluminum, wherein said silicon and magnesium are uniformly distributed throughout said alloy and are dissolved therein;
- (b) extruding said alloy at a temperature in excess of 950° F.; and
- (c) rapidly cooling said extruded alloy to a temperature of at least 350° F. in at most 4 minutes.

2. The process which comprises:

- (a) providing an aluminum base alloy consisting essentially of from 0.60 to 0.90 percent silicon, from 0.40 to 0.60 percent magnesium and the balance aluminum, wherein said silicon and magnesium are uniformly distributed throughout the said alloy;
- (b) heating said alloy to a temperature of at least 970° F.;
- (c) holding said alloy at said temperature of at least 970° F. for at least 2 minutes;
- (d) extruding said alloy at a temperature in excess of 950° F.; and
- (e) rapidly cooling said extruded alloy to a temperature of at least 350° F. in at most 4 minutes.

3. A process according to claim 2 where said silicon and magnesium are uniformly distributed throughout the said alloy by homogenizing at a temperature of from 970° to 1100° F. for from 4 to 20 hours.

10

20

25

30

4. A process according to claim 2 wherein after said rapid cooling said alloy is thermally artificially aged.

5. A process according to claim 4 wherein said artificial aging is from 15 minutes to 9 hours at 200 to 410° F.

6. A process according to claim 4 wherein said alloy is artificially aged at about 350° F. for from 4 to 8 hours.

7. A process according to claim 2 wherein the total silicon and magnesium content in said aluminum alloy is from 1.3 to 1.5 percent.

8. A process according to claim 2 wherein the ratio of silicon to magnesium in said aluminum alloy is from 1.30:1 to 1.5:1.

9. A process according to claim 2 wherein the alloy contains in addition 0.35 percent maximum iron, 0.10 percent maximum copper, 0.10 percent maximum manganese, 0.10 percent maximum chromium, 0.10 percent maximum zinc, 0.10 percent maximum titanium and 0.05 percent maximum each of other elements totaling a maximum 0.15 percent.

References Cited by the Examiner

UNITED STATES PATENTS

|           |         |               |          |
|-----------|---------|---------------|----------|
| 1,472,739 | 10/1923 | Archer et al. | 148—32.5 |
| 3,019,144 | 1/1962  | Murphy et al. | 148—12.7 |
| 3,113,052 | 12/1963 | Schneck       | 148—11.5 |

DAVID L. RECK, Primary Examiner.

30 H. F. SAITO, Assistant Examiner.